

Dec. 8, 1964

J. E. BROWN

3,160,592

ENGINE OPERATION AND COMPOSITIONS THEREFOR

Filed Oct. 16, 1959

FIGURE 1



INVENTOR.  
JEROME E. BROWN

BY  
*Kenneth Swartwood*

1

3,160,592  
ENGINE OPERATION AND COMPOSITIONS  
THEREFOR

Jerome E. Brown, Detroit, Mich., assignor to Ethyl Corporation, New York, N.Y., a corporation of Virginia

Filed Oct. 16, 1959, Ser. No. 847,018  
11 Claims. (Cl. 252—49.7)

This invention relates to a method of operating a spark ignition internal combustion engine which utilizes novel compositions of matter containing certain non-ionic metal polycarbonyl compounds which enable an engine to give knock-free performance and which possess numerous benefits in connection with improved combustion characteristics and the alleviation of modern day engine problems.

Concurrent with the development of the modern high efficiency, high compression ratio, internal combustion engine of the spark ignition type, it was necessary to develop fuels which would permit the knock-free operation required to utilize most effectively these advances in engine design. The approach to this problem has been in two directions. On the one hand, improvements in refining operations have been undertaken to provide hydrocarbon fuels, wherein the ingredients or mixtures thereof possess high antiknock quality. There exists, however, a limit, depending on a number of factors, beyond which the fuels cannot be economically improved. On the other hand, additives have been provided for such fuels whereby a further increase in the antiknock quality of the mixture is produced.

The most successful antiknock additive from a practical standpoint has been tetraethyllead. From time to time, a number of other antiknock materials have been proposed, but none of them has attained commercial significance in this country.

It is an object of this invention to provide an improved method for operating an internal combustion engine. Another object is to provide new compositions of matter. A more specific object is to provide new gasoline compositions. It is also an object of this invention to provide a gasoline containing certain metal polycarbonyl antiknock compounds or mixtures of such compounds which possess greatly reduced wear causing characteristics. A still further object is to provide gasoline suitable for use in high efficiency, spark ignition internal combustion engines requiring a fuel of high antiknock quality. Still another object is to provide a lubricating oil which acts to reduce the octane requirement of an internal combustion engine. Among the other objects of this invention is the alleviation of engine problems including octane requirement increase, spark plug fouling and surface ignition. Additional objects of the instant invention will be apparent from the discussion which follows:

The above and other objects of this invention are accomplished by providing a process for operating a spark ignition internal combustion engine which comprises introducing into the cylinders thereof, certain non-ionic manganese polycarbonyl antiknock agents defined below. The objects of this invention are also accomplished by providing, as novel compositions of matter, gasoline, lubricating oil and antiknock fluids containing said non-ionic manganese polycarbonyl compounds or mixtures of said manganese polycarbonyl compounds as antiknock agents.

2

Thus, among the important compositions contemplated by the present invention are included a hydrocarbon fuel of the gasoline boiling range for use in spark ignition internal combustion engines containing a small amount of non-ionic manganese polycarbonyls of the type defined sufficient to improve the antiknock properties of said hydrocarbon fuel. For most purposes this amount of manganese compound will range from about 0.01 gram to about 6 grams of manganese per gallon of fuel. In a preferred embodiment of the invention the amount of manganese compound is regulated so as to be equivalent to from 0.2 gram to 4 grams of manganese per gallon. More specifically, the present invention contemplates a hydrocarbon of the gasoline boiling range for use in spark ignition internal combustion engines containing substantially 1.77 grams of manganese in the form of a non-ionic manganese polycarbonyl of the type defined per gallon of fuel. Further compositions which are contemplated by the present invention include antiknock fluids which consist of organolead antiknock agents, usually alkyllead compounds such as tetraethyllead, together with non-ionic manganese polycarbonyls of the type defined. Also within the purview of the invention are gasolines containing mixtures of said organolead compounds and said manganese polycarbonyls. Both the fuels and the antiknock fluids may contain additional ingredients such as halogenated hydrocarbon scavengers, phosphorus deposit modifying compositions, antioxidants such as alkylated phenols and the like. The present invention also embraces the process of obtaining improved operating characteristics of a spark ignition internal combustion engine which comprises operating said engine on a fuel composition which consists of a hydrocarbon fuel of the gasoline boiling range containing a small amount of non-ionic manganese polycarbonyl sufficient to improve the antiknock properties of said hydrocarbon fuel.

Among the manganese carbonyl compounds suitable for use in the present invention are those which have the empirical formula  $R_xMn(CO)_y$  where R is an organic radical, x is 1 and y is 5. These compounds and their usefulness as antiknock agents are described in my copending application, Serial No. 683,759, now Patent Number 2,913,413, filed September 13, 1957, of which this application is a continuation-in-part. Application Serial No. 683,759 is in turn a continuation-in-part of my earlier copending application, Serial No. 645,828, now abandoned. R is most preferably a monovalent hydrocarbon radical, such as an alkyl or aryl radical, or a monovalent acyl radical. Examples of these compounds include methyl manganese pentacarbonyl, benzoyl manganese pentacarbonyl, phenyl manganese pentacarbonyl, acetyl manganese pentacarbonyl, and the like. These and other manganese polycarbonyl compounds exhibit extraordinary antiknock effect and other unexpected properties which render them of interest as commercial antiknock agents.

The relative size of the organic radical in the manganese carbonyl compounds, while not too important, is best limited to those having from 1 to about 20 carbon atoms, as it is found that these are best suited to the practice of this invention. Compounds having organic groups containing from 1 to 13 carbon atoms are preferred as these compounds are found to best combine the qualities of volatility and inductibility which are prerequisites to proper functioning as gasoline additives.

Compounds having the formula  $RMn(CO)_5$  where the

R represents an organic radical from the group consisting of organic hydrocarbon radicals and organic oxygen containing radicals, are conveniently prepared from manganese carbonyl in an ether solution. Manganese carbonyl is first converted to an alkali metal salt such as the sodium salt by treating the solution with an alkali metal present by an alkali metal dispersion or amalgam. The alkali metal salt is then reacted with an alkylating agent such as a dialkyl sulphate to form an alkyl manganese pentacarbonyl. Alternatively, the alkali metal salt of manganese carbonyl is reacted with an acyl halide to form an acyl manganese pentacarbonyl compound. These acyl manganese pentacarbonyl compounds are converted to the corresponding lower alkyl or aryl manganese pentacarbonyl compounds by pyrolysis accompanied by the loss of CO at elevated temperatures. Thus, phenyl manganese pentacarbonyl is conveniently produced by the pyrolysis of benzoyl manganese pentacarbonyl.

The lowest molecular weight compound having the formula  $RMn(CO)_5$  is methyl manganese pentacarbonyl which is a crystalline solid melting at about 95° C. and which is highly volatile and soluble in gasoline. Another compound of this class is benzoyl manganese pentacarbonyl, also a soluble crystalline solid, which melts at about 38° C. Propyl manganese pentacarbonyl and acetyl manganese pentacarbonyl are other representative members.

It is essential that the manganese polycarbonyl compounds used in the practice of this invention be non-ionic in nature in order that they produce the desired effect. For example, ionic manganese carbonyl compounds such as those having halogen bonded directly to manganese are not sufficiently volatile to be readily inducible into the cylinders of a multi-cylinder engine using a manifold type intake valve. These compounds are unable to give the benefits attributable to non-ionic manganese polycarbonyl compounds.

An unexpected feature of this invention is that the non-ionic manganese polycarbonyls are among the most effective antiknock agents tested to date. This is particularly surprising when it is considered that manganese is located in the Periodic Table next to the element chromium. Chromium carbonyl exhibits a pro-knock effect when employed as a gasoline additive for use in a spark ignition internal combustion engine.

Even when a compound has exceptional antiknock activity, the chances of its becoming a useful product remain extremely remote. This is due to the fact that many other properties must be taken into consideration before a new product can be seriously considered as a useful product. Thus, in the past, compounds having antiknock activity have been rejected from the commercialization because they

(a) Have a deleterious effect on the operation of an engine

(b) Are not sufficiently soluble in the fuel

(c) Are not volatile enough for proper engine inducibility

(d) Possess objectionable odors

(e) Bring about excessive wear

For example, various iron and nickel compounds including iron carbonyl and dicyclopentadienyl nickel have been suggested as antiknocks but have not been accepted due to the excessive engine wear caused by their use. As a further example, many aromatic amines exhibit antiknock activity, but their use is not feasible due to the fact that they exude a particularly objectionable odor.

Therefore, to be commercially successful, an antiknock must possess many auxiliary properties in addition to outstanding antiknock activity. Any compound under consideration must undergo extensive tests to insure that it meets the important secondary qualifications.

It has been found that the non-ionic manganese polycarbonyl compounds which are the subject of the present

invention, possess all the requirements of a successful antiknock to a remarkable degree. That is, they not only exhibit outstanding antiknock effectiveness, but in addition have the properties (including volatility, gasoline solubility, lack of gum forming tendencies, minimization of engine deposits and engine wear and susceptibility to preparation from available materials) required of commercial additives.

The fuels and lubricants used in today's high compression automotive engines cause deposits to be formed during combustion. These deposits which are derived from the fuels and lubricating oils and the additives therein collect on essentially all parts of the combustion chamber including the valves, the spark plugs and the cylinder walls. The formation of these deposits leads to several problems such as octane requirement increase, deposit induced ignition and spark plug fouling. These problems prevent maximum utilization of the potential of a fuel and limit the designer from providing engines which will accomplish this end.

Not only do the non-ionic manganese polycarbonyl compounds of this invention exhibit the properties required of a successful antiknock, but they also have valuable and unexpected auxiliary effects on the operation of a spark ignition internal combustion engine. It has been found that these compounds when used either as fuel or lube oil additives, minimize octane requirement increase and deposit induced ignition and increase the spark plug life of the modern high compression spark ignition internal combustion engine.

An important embodiment of this invention is gasoline containing, in amounts sufficient to improve the octane quality thereof, a non-ionic manganese polycarbonyl compound which is soluble in the gasoline. It has been found that non-ionic manganese polycarbonyl compounds are of outstanding effect as antiknock agents. The amount of the manganese polycarbonyl compound present in the compositions of this invention is regulated such that at least about 0.01 gram of manganese is present per gallon of the finished gasoline, and ordinarily up to about 6 grams of manganese per gallon is provided. In a preferred embodiment the amount of manganese polycarbonyl is regulated to provide from 0.2 gram to 4.0 grams of manganese per gallon of fuel.

The upper limit of beneficial use of the non-ionic manganese polycarbonyl compounds is, as a practical matter, limited due to the fact that at high concentrations the magnitude of the octane number benefit obtainable per unit weight of compound decreases to some extent. Thus, the most beneficial antiknock effect of the non-ionic manganese polycarbonyl compound is realized when these compounds are employed in concentrations such that there is from about 0.03 to about 10 grams of manganese per gallon of the finished gasoline. At higher concentrations the antiknock effect per unit weight is diminished, and the other beneficial effects are also reduced. When used as a primary additive, the best results are obtained when from about 0.01 to about 6 grams of manganese are present in the gasoline.

As the non-ionic manganese polycarbonyl compounds find outstanding and unexpected utility as additives to both gasoline and crankcase lubricating oil, this invention gives rise to novel compositions of matter comprising a liquid hydrocarbon mixture useful in a spark ignition internal combustion engine, which mixture contains a non-ionic manganese polycarbonyl compound of the type defined in amount sufficient to improve the combustion characteristics of the engine.

The non-ionic manganese polycarbonyl antiknock agents of this invention are also conveniently introduced into the cylinders of an internal combustion engine by utilizing a separate system of supply in conjunction with the system which supplies fuel to the cylinders. Thus, the non-ionic manganese polycarbonyl compounds are

supplied to the cylinders by atomizing, vaporizing or directly spraying the compound or a solution thereof, directly into the cylinders or into the intake manifold which supplies the cylinders with fuel. Introduction of the non-ionic manganese polycarbonyl compound into the manifolding system may be accomplished either prior or subsequent to carburetion or injection of the gasoline. When the non-ionic manganese polycarbonyl compound is a solid, it is often possible to vaporize it by passing a stream of air over or through a supply of the compound. When the compound is a liquid, it is conveniently supplied to the intake manifold through a wick which is supplied from a reservoir of the liquid.

FIGURE 1 is illustrative of a method of introducing a non-ionic manganese polycarbonyl compound into a combustion chamber of an internal combustion engine having a plurality of combustion chambers equipped with movable pistons wherein the walls of the chambers are lubricated with a crankcase lubricating oil and wherein gasoline is introduced into the combustion chamber and ignited and the products of combustion act upon the pistons and produce a driving force. With reference to FIGURE 1, the numeral 10 generally represents a cylinder and cylinder head of a multi-cylinder spark ignition internal combustion engine which contains a piston 11, combustion chamber 12, spark plug 13 which is under the influence of an ignition system (not shown), intake valve 14 and intake port 15 through which gasoline and combustion air are supplied by a carburetion system (not shown), an exhaust valve 16 and an exhaust port 17. These components make up the basic parts required in a conventional four-cycle spark ignition internal combustion engine.

To effectively conduct the process of this invention, a non-ionic manganese polycarbonyl compound is conveniently injected into the combustion chamber 12 by the utilization of a separate system which consists of a supplemental opening 18 which has fitted thereto a valve 19 shown for purposes of illustration as a poppet valve held closed by a spring 20 and having an elongated stem 21 which places the valve under the influence of a solenoid 22. The solenoid 22 is conveniently arranged to be under the influence of a set of breaker points (not shown) coordinated with the ignition system of the engine so that the valve 19 will be open during the intake stroke of the piston 11 for a time sufficient to permit the required amount of non-ionic manganese polycarbonyl compound to enter the combustion chamber 12. The non-ionic manganese polycarbonyl compound is supplied through the opening 18 by means of a vaporizing system 23 which terminates in an inlet port 24 through which the valve stem 21 operates by means of the aperture 25. The valve stem 21 is sealed in the aperture 25 in any convenient manner. To supply a non-ionic manganese polycarbonyl compound as a vapor to the combustion chamber 12 through the opening 18, a reservoir 26 of any convenient form contains a supply of manganese polycarbonyl compound to a convenient level 27. The container 26 is fitted with a means for passing vaporizing gas through the manganese polycarbonyl compound as shown by the conduit 28 which is attached to an opening 29 in the container 26. Back-up in the conduit 28 is prevented by any convenient means, such as a diaphragm valve 30. To the upper portion of the container 26 is attached a plurality of conduits 31 corresponding to the number of cylinders in the engine. The conduits 31 terminate in the inlet port 24. A vaporizing gas, such as nitrogen, air, carbon dioxide and the like, supplied from any convenient means such as a compressor or tank (not shown) through the conduit 28 passes through the manganese polycarbonyl compound 27 and carries the compound as a vapor through the conduit 31 to the inlet port 24 where at the appropriate time it passes through the aperture 18 into the combustion chamber 12 where it mixes with the gasoline and combustion air and improves the combustion which takes place under

the influence of spark plug 13 at the end of the compression stroke of the piston 11. The manganese polycarbonyl compound shown at 27 may be in the form of a solid such as methyl manganese pentacarbonyl or may be a liquid which contains a non-ionic manganese polycarbonyl which may be blended with an antiknock fluid containing halogen scavenger material and an organolead antiknock agent such as tetraethyllead.

Fuels containing organolead antiknock agents ordinarily contain, in addition to the antiknock agent, corrective agents commonly termed scavengers. Thus, when organolead antiknock agents are present in the compositions of this invention, it is desirable to include therewith such scavengers. These scavengers consist of organo bromine and/or chlorine compounds such as ethylene dibromide, ethylene dichloride and like material. They function to inhibit the build-up of lead deposits on the interior surface of internal combustion engines.

Halogen containing hydrocarbons are useful as scavengers in conjunction with the manganese polycarbonyl antiknock agents and are conveniently blended therewith to form fluids which are added to gasoline to give the benefits of this invention. These fluids also may contain small amounts of such hydrocarbon solvents as kerosene as well as dyes, antioxidants and the like. The proportion of halogen in such compositions is adjusted such that an atom ratio of halogen to manganese of from about 0.2:1 up to 12:1 is achieved. However, the octane enhancement of the manganese polycarbonyl compounds is realized even in the absence of such scavengers.

Organolead antiknock agents are commonly provided as fluids for addition to hydrocarbon fuels. These fluids ordinarily contain the organolead compound and the halogen scavenger agents referred to above. In addition, these fluids also often contain solvents comprising mixtures of hydrocarbons as well as antioxidants and the like. Thus, another variant within the purview of this invention is the provision of an antiknock fluid comprising an organolead compound and a manganese polycarbonyl compound. These fluids are conveniently blended with hydrocarbon fuels to prepare the improved fuels to this invention.

Because of the property inherent in the manganese polycarbonyl compounds within the scope of this invention of being highly soluble in gasoline, such blending operations present little or no difficulties. It is generally necessary only to add the requisite quantity of an improved antiknock fluid of the present invention to gasoline; and, by stirring, shaking or otherwise mechanically agitating these components, homogeneous improved fuel compositions are obtained. As a result of the high solubility of the antiknock fluids of this invention in gasoline such fluids can be utilized in any commercially available gasoline including straight run, catalytically cracked, catalytically reformed and thermally cracked base stocks and likewise, blends thereof.

In order to illustrate the utility and some of the commercial advantages of employing the manganese carbonyl compounds used in the practice of this invention, a great number of tests have been conducted. The results of some of the most significant are presented below.

A most important feature of the present invention is the outstanding antiknock activity exhibited by the non-ionic manganese polycarbonyl compounds.

To demonstrate this antiknock effectiveness, tests were made on gasolines both with and without these additives present. The tests were conducted on a single-cylinder CFR standard test engine according to the American Society for Testing Materials, Procedure D-908-55 (Research Method). The results of these tests are summarized in Table I from which it can be seen that the addition of a relatively small quantity of an organo manganese pentacarbonyl, such as methyl manganese pentacarbonyl, greatly improves the octane number of the gasoline.

## EXAMPLES II-VIII

Other improved gasoline compositions of this invention prepared as in Example I are illustrated in Table II. The initial boiling points (IBP) and final boiling points (FBP) of the gasolines used are indicated as well as the particular manganese polycarbonyl compounds and their concentrations in terms of grams of manganese per gallon of gasoline. Other such improved gasoline compositions will be apparent to one skilled in the art.

7 TABLE I

## Antiknock Effectiveness of Compounds of This Invention

| Additive                                | Octane Number of Gasoline with No Additive | Mn, g. per gal. | Resulting Octane Number |
|-----------------------------------------|--------------------------------------------|-----------------|-------------------------|
| Methyl manganese pentacarbonyl          | 91.8                                       | 0.18            | 93.1                    |
| Methyl manganese pentacarbonyl          | 91.8                                       | 0.26            | 93.8                    |
| Methyl manganese pentacarbonyl          | 91.8                                       | 1.0             | 96.0                    |
| Methyl manganese pentacarbonyl          | 91.8                                       | 2.0             | 97.1                    |
| Methyl manganese pentacarbonyl          | 91.8                                       | 3.0             | 99.9                    |
| Methyl manganese pentacarbonyl          | 91.8                                       | 0.59            | 94.6                    |
| Benzyl manganese pentacarbonyl          | 91.8                                       | 0.58            | 94.3                    |
| Acetyl manganese pentacarbonyl          | 91.8                                       | 0.28            | 92.9                    |
| Acetyl manganese pentacarbonyl          | 91.8                                       | 0.47            | 94.0                    |
| Acetyl manganese pentacarbonyl          | 91.8                                       | 1.0             | 95.5                    |
| Trifluoroacetyl manganese pentacarbonyl | 98.7                                       | 0.25            | 99.4                    |
| Trifluoroacetyl manganese pentacarbonyl | 98.7                                       | 1.0             | 101.0                   |
| Trifluoroacetyl manganese pentacarbonyl | 98.7                                       | 2.0             | 103.3                   |
| Methyl manganese pentacarbonyl          | 80                                         | 1.02            | 94.3                    |
| Methyl manganese pentacarbonyl          | 80                                         | 2.01            | 100.0                   |
| Propionyl manganese pentacarbonyl       | 91.8                                       | 0.28            | 94.5                    |
| Propionyl manganese pentacarbonyl       | 91.8                                       | 0.56            | 95.3                    |
| Phenyl manganese pentacarbonyl          | 91.8                                       | 0.50            | 94.4                    |
| Phenyl manganese pentacarbonyl          | 91.8                                       | 1.0             | 95.9                    |

The antiknock properties of manganese polycarbonyl compounds are even more unexpected when it is considered that some other compounds of manganese are ineffective. For example, manganese naphthenate exhibits a slight pro-knock quality.

The following examples are illustrative of the novel gasolines, lubricating oils and antiknock fluids which are within the scope of this invention.

## EXAMPLE I

A typical method of providing fuels containing a dissolved manganese polycarbonyl compound is as follows: To a gasoline having a final boiling point of 406° in a vessel provided with an agitator is added 6.29 parts of ethyl manganese pentacarbonyl per gallon of the gasoline. After agitating the mixture for approximately fifteen minutes, the ethyl manganese pentacarbonyl is completely dissolved and uniformly distributed throughout the fuel. This is demonstrated by analysis of a portion of the fuel for manganese, which shows the fuel to contain 1.77 grams of manganese per gallon of fuel mixture.

10

30

40

45

8 TABLE II  
Gasoline Containing Manganese Polycarbonyl Compounds

| Example | Gasoline |     | Manganese Polycarbonyl Compound       | Grams Mn per gal. |
|---------|----------|-----|---------------------------------------|-------------------|
|         | IBP      | FBP |                                       |                   |
| II      | 90       | 406 | Phenylacetyl manganese pentacarbonyl. | 0.01              |
| III     | 94       | 390 | Benzoyl manganese pentacarbonyl.      | 10.0              |
| IV      | 94       | 390 | Acetyl manganese pentacarbonyl.       | 6.0               |
| V       | 84       | 392 | Ethyl manganese pentacarbonyl.        | 0.1               |
| VI      | 89       | 385 | Methyl manganese pentacarbonyl.       | 2.0               |
| VII     | 93       | 378 | Acryl manganese pentacarbonyl.        | 4.0               |
| VIII    | 94       | 390 | Propionyl manganese pentacarbonyl.    | 1.8               |

## EXAMPLES IX-XIX

Table III illustrates typical gasolines of this invention which contain a non-ionic manganese polycarbonyl compound in conjunction with an organolead compound.

The organolead antiknocks which are ingredients of certain of the compositions of this invention are preferably hydrocarbon lead compounds such as tetraphenyllead, tetratolyllead and particularly tetraalkyllead compounds such as tetramethyllead, tetraethyllead, tetrapropyllead, and the like. Tetraethyllead is preferred. In general, the amount of organolead antiknock agent is selected so that its content of the gasoline is equivalent to about 0.1 to about 8 grams of lead per gallon of gasoline.

9 TABLE III  
Improved Gasolines Containing a Lead Antiknock Agent and a Non-Ionic Manganese Polycarbonyl Compound

| Example | Gasoline  |     |                | Manganese Polycarbonyl Additive          | Manganese, g./gal. | Lead Antiknock Agent | Grams of Pb per gal. | Scavenger            | Scavenger Conc., g./gal. |
|---------|-----------|-----|----------------|------------------------------------------|--------------------|----------------------|----------------------|----------------------|--------------------------|
|         | Percent S | FBP | Gravity, ° API |                                          |                    |                      |                      |                      |                          |
| IX      | 0.02      | 426 | 61.4           | Benzyl manganese pentacarbonyl.          | 0.25               | Tetraethyllead       | 3.17                 | (Ethylene dichloride | 1.48                     |
| X       | 0.02      | 426 | 61.4           | Trifluoromethyl manganese pentacarbonyl. | 0.1                | do                   | 3.17                 | (Ethylene dibromide  | 1.5                      |
| XI      | 0.02      | 426 | 61.4           | Methyl manganese pentacarbonyl.          | 6.0                | do                   | 3.17                 | (Ethylene dichloride | 1.48                     |
| XII     | 0.03      | 390 | 59.0           | p-Octyl benzyl manganese pentacarbonyl.  | 2.4                | Tetramethyllead      | 2.0                  | (Ethylene dibromide  | 1.5                      |
| XIII    | 0.065     | 366 | 54.6           | Nonoyl manganese pentacarbonyl.          | 4.0                | Tetraphenyllead      | 0.05                 | Dibromobutane        | 2.1                      |
| XIV     |           | 385 | 64.4           | Acetyl manganese pentacarbonyl.          | 0.03               | Tetraethyllead       | 8.00                 | Ethylene dichloride  | 4.3                      |
| XV      |           | 420 | 61.4           | Benzoyl manganese pentacarbonyl.         | 8.0                | Tetrabutyllead       | 0.1                  | (Dibromotoluene      | 1.4                      |
| XVI     |           | 416 | 63.2           | Phenyl manganese pentacarbonyl.          | 0.9                | Tetraethyllead       | 5.1                  | 62 Mix               |                          |
| XVII    | 0.02      | 426 | 61.4           | Methyl manganese pentacarbonyl.          | 0.05               | do                   | 0.95                 | do                   |                          |
| XVIII   |           | 420 | 60.8           | Ethyl manganese pentacarbonyl.           | 0.10               | do                   | 0.90                 | do                   |                          |
| XIX     | 0.001     | 395 | 55.6           | Tolyl manganese pentacarbonyl.           | 0.30               | do                   | 2.70                 | do                   |                          |

Antiknock activity of mixtures of my manganese additives with organolead antiknocks is shown in Table IV.

TABLE IV

*Antiknock Effectiveness of Mixtures of Compounds of This Invention With Organolead Antiknock Agents*

| Organolead Agent,<br>3 ml./gal. | Manganese Additive               | Conc.,<br>g. Mn/<br>gal. | Octane No. of Fuel |                 |                 |
|---------------------------------|----------------------------------|--------------------------|--------------------|-----------------|-----------------|
|                                 |                                  |                          | Clear              | Organolead Only | Organolead + Mn |
| TEL-----                        | Methyl manganese pentacarbonyl.  | 0.05                     | 89.0               | 97.9            | 98.5            |
| TEL-----                        | Methyl manganese pentacarbonyl.  | 0.5                      | 89.0               | 97.9            | 99.0            |
| TEL-----                        | Methyl manganese pentacarbonyl.  | 1.0                      | 89.0               | 97.4            | 101.3           |
| TEL-----                        | Methyl manganese pentacarbonyl.  | 1.0                      | -----              | 99.3            | 101.4           |
| TML-----                        | Methyl manganese pentacarbonyl.  | 1.0                      | -----              | 92.5            | 98.7            |
| TEL-----                        | Benzoyl manganese pentacarbonyl. | 1.0                      | 89.0               | 97.5            | 98.7            |
| TEL-----                        | Trifluoromethyl pentacarbonyl.   | 0.1                      | 89.0               | 97.1            | 97.9            |
| TEL-----                        | Trifluoromethyl pentacarbonyl.   | 1.0                      | 89.0               | 97.1            | 98.9            |

TEL=tetraethyllead. TML=tetramethyllead.

Other compositions of this invention comprising an improved gasoline containing a non-ionic manganese polycarbonyl compound are prepared in a manner similar to that described above and illustrated in Examples I through XIX. Further, illustrative examples of the non-ionic manganese polycarbonyl compounds utilized alone or in admixture in such improved gasolines include propionyl manganese pentacarbonyl, phenyl manganese pentacarbonyl, benzoyl manganese pentacarbonyl, benzyl manganese pentacarbonyl, m-ethylbenzyl manganese pentacarbonyl and the like.

Where halohydrocarbon compounds are employed as scavenging agents, the amounts of halogen used are given in terms of theories of halogen. A theory of halogen is defined as the amount of halogen which is necessary to react completely with the metal present in the antiknock mixture to convert it to the metal dihalide, as, for example, lead dihalide and manganese dihalide. In other words, a theory of halogen represents two atoms of halogen for every atom of lead and/or manganese present. In like manner, a theory of phosphorus is the amount of phosphorus required to convert the lead present to lead orthophosphate,  $Pb_3(PO_4)_2$ , that is, a theory of phosphorus based on lead represents an atom ratio of two atoms of phosphorus to three atoms of lead. When based on manganese, a theory of phosphorus likewise represents two atoms of phosphorus for every three atoms of manganese, that is sufficient phosphorus to convert manganese to manganese orthophosphate,  $Mn_3(PO_4)_2$ .

The scavenger compounds can be halohydrocarbons both aliphatic and aromatic in nature, or a combination of the two, with halogens being attached to carbons either in the aliphatic or the aromatic portions of the molecule. The scavenger compounds may also be carbon, hydrogen and oxygen-containing compounds, such as haloalkyl ethers, halohydrins, halo esters, halonitro compounds, and the like. Still other examples of scavengers that may be used in conjunction with my manganese compounds either with or without hydrocarbolead compounds are illustrated in U.S. Patents 2,398,281 and 2,479,900-903, and the like. Mixtures of different scavengers may also be used. These fluids can contain other components as stated hereinabove. In like manner, manganese-containing fluids are prepared containing from 0.01 to 1.5 theories of phosphorus in the form of phosphorus compounds. To make up the finished fuels, the concentrated fluids are added to the gasoline in the desired amounts and the homogeneous fluid obtained by mixing, agitation, etc.

30

35

50

55

60

65

70

75

added 5 parts of ethylene dichloride and the mixture agitated until a homogeneous fluid results. The manganese to chlorine atom ratio in this fluid is 1:12 and represents 6 theories of halogen based on the manganese.

In like manner, a fluid is prepared comprising benzyl manganese pentacarbonyl and ethylene dibromide in which the manganese to bromine ratio is 1:6, representing 3 theories of bromine based on the manganese. Likewise, a fluid containing isobutyryl manganese pentacarbonyl, ethylene bromohydrin, and 2,3-dichloro 1,4-dimethylbenzene is prepared in such proportions that for every 75 atoms of manganese, there are one atom of bromine and two atoms of chlorine, representing a total of 0.02 theory of halogen.

The above fluids are added to hydrocarbon fuels in amounts so as to provide improved fuels containing 0.015 gram, 0.25 gram, 1.00 gram, 6 grams and 10 grams of manganese per gallon.

## EXAMPLE XXI

To 8.0 parts of lead in the form of tetraethyllead in an antiknock fluid containing 0.5 theory of bromine as ethylene dibromide and 1.0 theory of chlorine as ethylene dichloride, wherein the theories of halogen are based upon the amount of lead present, is added 0.015 part of manganese in the form of an equimolar mixture of benzyl manganese pentacarbonyl and acetyl manganese pentacarbonyl.

This fluid is then added to a commercial hydrocarbon fuel having an initial boiling point of 82° F. and a final boiling point of 420° F. in an amount so as to provide 8.0 grams of lead and 0.015 gram of manganese per gallon.

## EXAMPLE XXII

A concentrated fluid is prepared as in Example XX containing kerosene, a blue dye, and 10 parts by weight of manganese as an equimolar mixture of methyl manganese pentacarbonyl and benzoyl manganese pentacarbonyl for every 0.02 part of lead in the form of diethyldimethyllead. This fluid is then blended with a commercial hydrocarbon fuel having an initial boiling point of 90° F. and a final boiling point of 394° F. in an amount sufficient to provide 10 grams of manganese and 0.02 gram of lead per gallon.

## EXAMPLE XXIII

Tetraethyllead and manganese pentacarbonyl are admixed so that the ratio is 2.0 grams of lead as tetraethyllead present for every 1.0 gram of manganese present

as phenyl manganese pentacarbonyl. This composition is found to possess superior antiknock and deposit modifying properties when added to gasoline.

## EXAMPLE XXIV

To the composition of Example XXIII is added ethylene dibromide in amount such that there is one theory of scavenger present based upon the total amount of metal.

The amount of the improved antiknock fluids of this invention containing organolead compounds and manganese polycarbonyl compounds employed in gasoline is dependent primarily upon the use for which the gasoline is intended. In gasolines for use in automotive engines, such as passenger cars, trucks, buses and the like, amounts of any of the compositions of this invention equivalent to from between about 0.1 and about 4.3 grams of lead per gallon are satisfactory. It will be appreciated, however, that in most cases the lead content of such improved fuels is preferably from between about 1.06 and about 3.17 grams of lead per gallon which, when the organolead constituent of such fuels is tetraethyllead, is equivalent to from between about 1 and about 3 milliliters of tetraethyllead per gallon. When the improved gasolines of this invention are designed primarily for use in aviation engines, somewhat greater concentrations can be tolerated and are frequently preferred. In such instances, it is advantageous to employ an amount of improved antiknock fluid of this invention equivalent to from between about 3.17 grams and about 6.34 grams of lead per gallon. That is to say, when utilizing a tetraethyllead-containing antiknock fluid of the present invention in an aviation fuel, amounts of such a fluid equivalent to from between about 3 and about 6 milliliters of tetraethyllead per gallon are satisfactory. Concentrations above these limits can be employed in both motor and aviation fuels, practical considerations being the prime criterion for establishing the upper concentration limit.

Use of antiknock fluids containing my non-ionic manganese polycarbonyls in addition to resulting in great convenience in storage, handling, transportation, blending with fuels, and so forth, also are unexpectedly potent concentrates which serve the multi-purpose functions of being useful as antiknocks, deposit modifiers, valve corrosion inhibitors, wear reducers, and the like. The fluids are also found to possess a surprising degree of inherent stability.

The gasolines to which the antiknock compositions of this invention are added are mixtures which may have a wide variation of compositions. These fuels can contain all types of hydrocarbons, including paraffins, both straight and branched chain; olefins; cycloaliphatics containing paraffin or olefin side chains; and aromatic containing aliphatic side chains. The gasoline type depends on the base stock from which it is obtained and on the method of refining. For example, it can be a straight run or processed hydrocarbon, including thermally cracked, catalytically cracked, reformed fractions, etc. When used for spark-fired engines, the boiling range of the components of gasoline can vary from zero to about 430° F., although the boiling range of the fuel blend is often found to be between an initial boiling point of from about 80° F. to 100° F. and a final boiling point of about 430° F. While the above is true for ordinary gasoline, the boiling range is a little more restricted in the case of aviation gasoline. Specifications for the latter often call for a boiling range of from about 82° F. to about 338° F., with certain fractions of the fuel boiling away at particular intermediate temperatures. All commercial gasolines including all those embraced within the present invention, always contain a great number of individual hydrocarbon compounds as components and always have a final boiling point of at least 300° F.

The gasolines in which the antiknock agents of this invention can be employed often contain minor quantities of various impurities. One such impurity is sulfur which can be present either in a combined form as an

organic or inorganic compound or as the elemental sulfur. The amounts of such sulfur can vary in various fuels from about 0.003 percent to about 0.30 percent by weight. Fuels containing quantities of sulfur, both lesser and greater than the range of amounts referred to above, are also known.

For best results in terms of spark plug life, the improved gasolines of this invention should contain at least 0.015 weight and 0.065 weight percent of this element. These gasolines may also contain organolead antiknock agents in the amounts specified above.

It will be apparent that the present invention is susceptible of additional variations. Some of these variants include the utilization in the antiknock fluid embodiments of solubilizing agents, such as kerosene, petroleum cuts or fractions, and in general various aromatic solvents including those containing diphenyl and the like. In addition to this, various organolead stabilizers can be used in such embodiments. Among such materials are included styrene, naphthalene, lecithin, aminodiphenyl amines, phenyl- $\alpha$ -naphthyl amine and analogous materials. Likewise, in both the antiknock fluid and anti-knock fuel embodiments of this invention it is frequently advantageous to employ minor proportions of antioxidants, particularly those of the phenylene diamine type as well as the various alkyl phenols, such as 2,6-di-*tert*-butyl phenol, 2,4,6-tri-*tert*-butyl phenol, o-*tert*-butyl phenol, etc. A still further variant within the contemplation of this invention relates to the utilization of various organic dyestuffs in the antiknock fluid embodiments of this invention, which materials serve primarily as a means of product identification, although frequently the coloration produced by such dyestuffs imparts to the composition a degree of stabilization against deterioration resulting from exposure to light. Furthermore, under certain circumstances benefits are to be obtained by utilizing as the scavengers in the diverse compositions of the present invention, organic halides possessing volatilities comparable to that of the organolead antiknock agent utilized. Such scavengers are described in several of the patents cited hereinbefore.

The improved gasolines and fluids of the present invention can be utilized in conjunction with other well known motor fuel adjuvants. Of such materials, the various catalytically active substances, such as phosphorus compounds comprising various phosphates, phosphites, phosphonates and the like can thus be used in various embodiments of this invention. Other variants within the contemplation of this invention will be apparent to those skilled in the art.

The manganese polycarbonyl containing additives of this invention may be mixed with antioxidants, such as alkylated phenols and amines, metal deactivators, phosphorus compounds; antiknock agents, such as amines as well as the alkyllead compounds mentioned above anti-rust and anti-icing agents, and wear inhibitors.

## EXAMPLE XXV

To 500 parts of a commercially available neutral crankcase lubricating oil is added a quantity of methyl manganese pentacarbonyl sufficient to produce a composition containing about 2.5 weight percent manganese. The mixture is agitated until the manganese pentacarbonyl is completely dispersed in the oil.

## EXAMPLE XXVI

To 10,000 parts of a wholly-distilled mixed base, solvent-refined lubricating oil having a gravity of 28.9° API, a viscosity grade of SAE 10W-20 and a viscosity index of 135.7 is added 100 parts of manganese as 2,4,6-triethylbenzyl manganese pentacarbonyl and the mixture is stirred until a homogeneous solution is obtained.

## EXAMPLE XXVII

To 1000 parts of a mixed-base, solvent-refined lubricating oil containing bright stock and which has an SAE

viscosity grade of 20, an API gravity of 30.5° and a viscosity index of 107.4 is added 0.05 percent manganese as benzyl manganese pentacarbonyl.

## EXAMPLE XXVIII

To 2162 parts of a wholly-distilled lubricating oil having an API gravity of 30.3°, a viscosity index of 154.2 and an SAE number of 5W-20 is added 10 percent manganese as benzoyl manganese pentacarbonyl and the mixture is stirred until the benzoyl manganese pentacarbonyl is dissolved.

## EXAMPLE XXIX

To 216 parts of a wholly-distilled lubricating oil having an API gravity of 29.1, an SAE number of 10W-30 and a viscosity index of 138.9 is added 3 percent of manganese as phenyl butyryl manganese pentacarbonyl. The mixture is agitated until a homogeneous solution is obtained.

The lubricating oils used in the practice of this invention include those fractions or blends of fractions from mineral oils which are used for lubricating purposes in the crankcase of an internal combustion engine. Lubricating oil stock is usually considered to include all the distillate obtainable from crude oils after the lower boiling fractions and gas oils have been expelled, as well as some of the residues that are left in the still when non-asphaltic crudes are distilled.

Generally lubricating oils are made from distilled fractions of a crude, but often these distilled fractions are combined with refined residuum, such as bright stocks, to yield oils having excellent lubricating qualities.

In addition to the non-ionic manganese pentacarbonyl compound, the lubricating oils of this invention may contain other additives. These other additives may include, for example, viscosity index improvers, detergents, corrosion inhibitors, metal deactivators, rust inhibitors, color stabilizers, pour depressants, emulsifiers, dyes, etc.

The non-ionic manganese polycarbonyl compounds used in the practice of this invention are prepared by various methods. Examples of these are indicated below.

## EXAMPLE XXX

Sodium manganese pentacarbonyl was prepared by treating a 5 percent solution of manganese carbonyl in tetrahydrofuran with an excess of one percent sodium amalgam. After removal of the excess amalgam, the supernatant liquid was treated with dimethyl sulfate and the resulting mixture, after standing overnight, was added to ice water and filtered. The precipitate was carefully dried in air and recrystallized forming a low-boiling petroleum ether to give a 59.5 percent yield of methyl manganese pentacarbonyl.

Similar methods are employed to give excellent yields of benzyl manganese pentacarbonyl, benzoyl manganese pentacarbonyl, styryl manganese pentacarbonyl and the like.

## EXAMPLE XXXI

Benzoyl manganese pentacarbonyl is prepared in a manner similar to that described in Example XXX by reacting benzoyl chloride with sodium manganese pentacarbonyl. The benzoyl manganese pentacarbonyl is gently heated to above 90° C. at which temperature a strong evolution of gas is readily identified as carbon monoxide. When the gas evolution ceases, the remaining product is found on analysis to be phenyl manganese pentacarbonyl.

## EXAMPLE XXXII

When 8.7 parts of  $\text{NaMn}(\text{CO})_5$  contained in 88 parts of tetrahydrofuran was treated with 3.2 parts of allyl chloride in a nitrogen atmosphere and the resulting mixture cautiously heated to reflux for one hour, the mixture became turbid. Removal of the solvent by distillation through a helix-packed column followed by distillation of the residues at reduced pressure gave a small yield

of pale yellow liquid (allyl manganese pentacarbonyl) which solidifies on cooling to ice bath temperature. The compound has a boiling point of 32° C. at 2 millimeters.

*Analysis.*—Calcd. for  $\text{C}_8\text{H}_5\text{MnO}_5$ : Mn, 23.3. Found: Mn, 23.5.

## EXAMPLE XXXIII

The sodium salt of 4.1 parts of manganese carbonyl was reacted with three parts of acetyl chloride to give 3.5 parts of a pale yellow solid melting between 43 and 48° C. This material was purified by successive sublimation to give 2.6 parts (a 51 percent yield) of pure acetyl manganese pentacarbonyl which melted at 54 to 56° C. Analysis of this compound showed that it contained 35.2 percent carbon, 1.28 percent hydrogen and 23.1 percent manganese. This corresponds very well with a calculated content of 35.32 percent carbon, 1.27 percent hydrogen and 23.17 percent manganese for the formula  $\text{CH}_3\text{COMn}(\text{CO})_5$ .

## EXAMPLE XXXIV

A solution of 21.8 parts of sodium manganese pentacarbonyl was prepared by reacting 19.5 parts of manganese pentacarbonyl in 133 parts of anhydrous tetrahydrofuran with an excess of freshly prepared one percent sodium amalgam under nitrogen in a reaction vessel. This solution was then transferred under nitrogen into a reaction vessel equipped with a stirrer, dropping funnel, reflux condenser and nitrogen sweep. To the stirring solution from the funnel was slowly added 31.5 parts of trifluoroacetic anhydride. An exothermic reaction occurred and a color change from opaque green/brown to an almost transparent yellow took place. The solution was allowed to stir overnight at room temperature after which it was poured into ice water. A pale yellow solid separated, was filtered off, and pressed dry. This yellow material, when recrystallized from carbon tetrachloride, gave 21.5 parts (81.4 percent yield) of white, fluffy crystalline product, perfluoroacetyl manganese pentacarbonyl having a melting point of 56.5-57.5° C.

## EXAMPLE XXXV

Two samples of perfluoroacetyl manganese pentacarbonyl, 3.1 parts and 2.0 parts respectively, were weighed separately into reaction vessels which were subsequently cooled and evacuated. The vessels were then heated carefully to the temperature of hot water, and then rapidly heated to 130-140° C. Both samples melted into yellow liquids and gas evolution was observed. Immediately after this evolution slowed, the vessels were cooled. Yellow-white solids covered the vessel interiors and these were recrystallized from carbon tetrachloride and combined to give a total of 2.9 parts (63.0 percent yield) of white crystalline perfluoromethyl manganese pentacarbonyl, M.P. 82-84° C. The infrared spectrum supported the proposed structure.

*Analysis.*—Calcd. for  $\text{C}_6\text{F}_3\text{O}_5\text{Mn}$ : Mn, 20.8. Found: Mn, 21.3.

When the non-ionic manganese polycarbonyl compounds used in the practice of this invention contain an organic radical, such radical has, in general, from 1 to about 20 carbon atoms. Thus, compounds suitable for use in the process of this invention include pelargonyl manganese pentacarbonyl, dibutyl manganese tetracarbonyl, methyl manganese pentacarbonyl, and the like. These compounds have a molecular weight from about 194 to about 500.

When the organic group is a hydrocarbon radical, it preferably has from 1 to about 13 carbon atoms and the manganese polycarbonyl compound which contains it has a molecular weight up to about 450. Examples of such non-ionic manganese polycarbonyl compounds include ethyl manganese pentacarbonyl, allyl manganese pentacarbonyl, phenyl manganese pentacarbonyl, p-hexyl benzyl manganese pentacarbonyl, and the like.

Likewise, when the organic group is an acyl radical or an acylated hydrocarbon radical, it preferably contains up to about 13 carbon atoms and the non-ionic manganese polycarbonyl compound has a molecular weight up to about 465. Examples of these compounds include benzoyl manganese pentacarbonyl, stearoyl manganese pentacarbonyl, and the like.

The present invention resides in the discovery that the non-ionic manganese polycarbonyl compounds are unexpectedly beneficial with regard to antiknock effect when used in conjunction with the operation of a spark ignition internal combustion engine. The invention gives rise to a number of embodiments including a novel process for operating such an engine by means of introducing a non-ionic manganese polycarbonyl compound into the combustion chambers, and a number of novel compositions which are of particular benefit in such a process. These novel compositions include a liquid hydrocarbon mixture for use in such an engine which mixture contains a non-ionic manganese polycarbonyl compound. This liquid hydrocarbon mixture, as has been pointed out, may be a gasoline or a lubricating oil. When the hydrocarbon is a gasoline it may contain an organolead antiknock agent and appropriate halohydrocarbon scavengers in addition to the manganese polycarbonyl compound. Suitable organolead compounds include the alkyllead compound, tetraethyllead, which may be present in amount such that up to 6.34 grams or more of lead are present per gallon of fuel. The atom ratio of manganese to lead may be from about 0.05 to 1 to 64 to 1, or, expressed differently, from about 1 to 20 to about 64 to 1. Applicable halohydrocarbon scavengers include ethylene dichloride and ethylene dibromide.

Further novel compositions of particular benefit in conducting the process of this invention comprise antiknock fluids containing a non-ionic manganese polycarbonyl. Fluids containing halohydrocarbon scavengers along with the non-ionic manganese polycarbonyl compound are also within the scope of this invention, as are fluids containing organolead antiknock agents in addition to the non-ionic manganese polycarbonyl compounds. Illustrative of such fluids are those containing methyl manganese carbonyl and tetraethyllead such that the atom ratio of manganese to lead is from about 0.05 to about 64 to 1. These fluids are conveniently added to gasolines to give compositions containing up to 6.34 or more grams of lead per gallon.

A variant in the practice of the present invention comprises the use of a non-ionic manganese polycarbonyl compound wherein the organic group is substituted with a non-ionic, non-reactive group.

Having fully described the nature of the present invention, the need therefor, and the best modes derived for carrying it out, it is intended that this invention be limited only within the spirit and scope of the appended claims.

I claim:

1. A liquid hydrocarbon crankcase lubricating oil containing from about 0.05 to about 10 weight percent manganese as a non-ionic manganese polycarbonyl compound having the formula

ganese as a non-ionic manganese polycarbonyl compound having the formula



wherein R is an organic radical selected from the group consisting of hydrocarbon radicals and acyl radicals and contains from 1 to about 20 carbon atoms.

2. The composition of claim 1 wherein R is an aliphatic hydrocarbon radical.

3. The composition of claim 1 wherein R is an aryl hydrocarbon radical.

4. The composition of claim 1 wherein R is an acyl radical.

5. Hydrocarbons of the gasoline boiling range containing from 0.01 to about 10 grams of manganese per gallon

15 as a non-ionic manganese polycarbonyl compound having the formula



wherein R is an organic radical selected from the group 20 consisting of hydrocarbon radicals and acyl radicals and contains from 1 to about 20 carbon atoms.

6. The composition of claim 5 wherein R is an aliphatic hydrocarbon radical.

7. The composition of claim 5 wherein R is an aryl hydrocarbon radical.

8. The composition of claim 5 wherein R is an acyl radical.

9. The composition of claim 5 additionally containing from about 0.1 to about 8.0 grams of lead per gallon

30 as an organo-lead antiknock agent.

10. An antiknock composition comprising a mixture of an organolead antiknock agent and a non-ionic manganese polycarbonyl compound having the formula



35 wherein R is an organic radical selected from the group consisting of hydrocarbon radicals and acyl radicals and containing from 1 to about 20 carbon atoms, wherein the atom ratio of manganese-to-lead is from about 1:20 to about 64:1.

11. Gasoline containing a small antiknock quantity of methyl manganese pentacarbonyl, said antiknock quantity being between equivalent to about 0.01 to about 10 grams of manganese per gallon.

45 References Cited in the file of this patent

UNITED STATES PATENTS

|           |              |                |
|-----------|--------------|----------------|
| 1,954,865 | Danner       | Apr. 17, 1934  |
| 2,398,282 | Bartholomew  | Apr. 9, 1946   |
| 2,434,578 | Miller       | Jan. 13, 1948  |
| 2,763,617 | Scott et al. | Sept. 18, 1956 |

FOREIGN PATENTS

|           |        |               |
|-----------|--------|---------------|
| 1,092,700 | France | Nov. 10, 1954 |
| 1,095,084 | France | Dec. 15, 1954 |

OTHER REFERENCES

"Journal of the Institute of Petroleum Technologists," vol. 13, 1927, pages 244-255.

69 "Journal of the American Chemical Society," vol. 71, 1949, page 1899.